

# United States Patent Office

2,952,607

Patented Sept. 13, 1960

1

2,952,607

## PROCESS FOR PRODUCING FUEL OILS HAVING IMPROVED RADIATION EMISSION

Warren C. Simpson, Berkeley, Calif., assignor to Shell Oil Company, New York, N.Y., a corporation of Delaware

No Drawing. Filed Sept. 15, 1958, Ser. No. 760,868

5 Claims. (Cl. 208—15)

The present invention relates to the operation of furnaces in which fluid fuels are burned. More particularly, it is concerned with a method of improving and controlling the radiant heat or emissivity of flames produced in furnaces.

In many types of furnaces wherein the fuel burned is oil, gas, or mixtures thereof, at least a part of the heat released by the flame is transferred from the flame to the body being heated by means of radiation. This either occurs directly, as in the case of a solid charge, or indirectly, as in the case of a liquid charge. Open hearth steel furnaces, lime and cement kilns, annealing furnaces, tube still heaters, cracking furnaces, and the like are examples of many types of furnaces largely dependent upon radiant heat transfer. The present invention is especially directed to the operation of open hearth furnaces in steel making processes, but the principles and process apply to these other types of furnaces as well.

In all of such types of furnaces, the proportion of heat transferred to the charge by radiation is largely fixed by the design of the furnace and by the characteristics of the flame. For example, in an open hearth furnace nearly all of the heat is transferred to the charge by radiation. In the usual case of a tube still heater or kiln to which the charge is continuously fed at a constant temperature and rate, the proportion of radiant heat transfer depends upon the ratio of the tube surface area which the flame "sees" to the tube surface area which is in contact with the combustion gases, but which the flame cannot "see." As long as outlet temperatures must remain constant at a predetermined value, which is almost always true, the heat absorption profile of the charge within the furnace has not heretofore been a variable, once a particular furnace design is selected and a particular fuel utilized.

Industrial furnaces are ordinarily extremely large capital investments and it is obvious that increased flexibility in the operation of such furnaces would be highly advantageous.

The copending application of which the present application is a continuation-in-part, Serial No. 641,874, filed February 25, 1957, now Patent No. 2,913,043, describes the improvement in radiation of residual fuel oils by precipitation of asphaltogenic bodies with relatively low molecular weight precipitants, such as kerosene, lower molecular weight paraffins down to and including butane and pentane. While these materials are satisfactory for the precipitation of the radiation emitting particles with which that and the present invention are both concerned, it will be realized that the use of such precipitants involves increased cost of fuel oil components, since kerosene and the lower hydrocarbons have a higher unit cost than the relatively inexpensive residual fuel oils.

Consequently, a major object of the present invention is to provide a method for controlling the radiation effect within furnaces at a lower cost than heretofore possible.

2

It is a more particular object of this invention to provide increased flexibility in the radiation effects of flames burning in the furnaces. It is a further object of the present invention to reduce the cost of operating such furnaces not only with respect to fuel components but with respect to the time necessary for causing the required degree of heating of the materials being subjected to the heat evolved in and by such furnaces. Other objects will become apparent during the following detailed discussion of the invention.

Now, in accordance with the present invention, it has been found that the radiation or emissivity (in the infrared spectral region) of a flame burned in a furnace may be increased by mixing two incompatible residual fuel oils, proportions thereof mixed in quantities at least sufficient to cause precipitation of high molecular weight asphaltogenic materials, namely, those having molecular weights above about 1,000 (preferably 1,000-5,000) present in at least one of the residual fuel oils and thereafter burning the fuel containing said particles, whereby flames of increased emissivity are obtained. The two residual fuel oils are employed in volume proportions between about 1:4 to about 4:1, and preferably are mixed in volume proportions of between about 25-75% and 75-25%.

More particularly, the present process comprises the mixing of at least two residual fuel oils, which each individually may show no evidence of precipitation of asphaltogenic particles therein, in such proportions that asphaltogenic particles are precipitated. The precipitation is based upon the relationship of the precipitating tendencies of the asphaltogenic materials present in the residual oils and the solution power of the cutter stock formed by the blend of two or more residual fuel oils containing the same.

Residual fuel oils generally (but not always) consist of a blend of vacuum flashed or thermally cracked residue oil in a mixture of lighter distillates commonly referred to as "cutter stocks" of relatively low viscosity. When the aromatic or heteroaromatic components of the residue having molecular weights greater than about 1000 are maintained in true solution by the lower molecular weight aromatics and heteroaromatics in the system, the fuel oil will be optically clear when examined in thin layers. When the solubilizing power of the lower molecular weight components of the residual fuel oil is not sufficient to maintain true solution, the occurrence of molecular association between various of the higher molecular weight polar components leads to the formation of loose aggregates of molecules into clusters which eventually grow into aggregates sufficiently large to be visible to the unaided eye as a precipitate. The principle effect of the present invention is to adjust the balance of precipitable materials with solvating materials in such a way as to cause the desirable type of precipitation for the purpose of later burning to effect an increase in radiation of the flame.

In the discussion of the aspects of the invention which follow, reference frequently will be made to two terms, namely, precipitation index and solvency index. The precipitation index is defined as the volume percentage concentration of alpha-methyl naphthalene plus residual fuel in a mixture with cetane that causes incipient precipitation of the residue. For this test a solution of the residue in alpha-methyl naphthalene is made containing about 10% residue. A small drop of this solution is taken with a wire or rod and placed on a piece of filter paper. (Smooth hard porous paper such as Whatman No. 50 is preferable.) This will normally soak into the paper and leave a fairly uniform brown area about  $\frac{1}{2}$  to  $\frac{3}{4}$  inch in diameter. If, however, a dark brown or black

ring or spot the size of the original drop remains, that indicates the presence of coke particles (as in the Oliensis test) and the solution should be filtered. One or two milliliters of the solution, filtered if necessary, is pipetted into a test tube or vial. Cetane (n-hexadecane) is added in measured increments to the measured volume of solution. After each increment is added the vial is stoppered, shaken, and a small drop of the solution removed and placed on the filter paper. The cetane is conveniently added from a 5 ml. buret, and the size of the increments will depend on the accuracy desired in the determination. A series of spots on filter papers will then be obtained representing solutions of the residue in a series of mixtures of alpha-methyl naphthalene and cetane.

Examination of these spots will reveal a certain ratio of the two solvents at which a darker ring or spot the size of the original drop is superimposed on the brown area on the filter paper. At higher cetane concentrations the ring or spot becomes more pronounced; at lower concentrations it is absent. The point at which the ring starts to appear, then, is that point at which the total mixture is of barely adequate aromaticity to dissolve the least soluble component of the residue. The volume percentage concentration of alpha-methyl naphthalene plus residue fuel in the total mixture with cetane that causes incipient precipitation of the residual fuel oil is designated as the "precipitation index" of that residue. It has been found that this value can usually be determined reproducibly to less than one unit.

Cutter stocks and solvents for asphaltogenic residues can be evaluated on the same basis as residues by this test method. In this case one or the other of the two standard solvents, namely, cetane or alpha-methyl naphthalene, as determined by preliminary test, is replaced by the cutter stock and a precipitation point is determined using a residue whose precipitation index has been found by the standard procedure. A residue or fraction of high asphaltene content relatively undiluted with non-asphaltic constituents is preferred as a standard for the test. Thus, a mixture of cutter stock in one standard solvent is found that is equivalent to a known mixture of alpha-methyl naphthalene and cetane with respect to a given residue or sample of asphaltenes, from which information the solvent power of the cutter stock can be expressed in terms of the volume percentage of alpha-methyl naphthalene in a mixture of the same with cetane that has the same solvent power as the cutter stock. This is termed the solvency index of the cutter stock.

Since the test as applied to residues measures the point of incipient precipitation of the least soluble component in relatively dilute solution, any addition of more soluble materials to a residue (or the more soluble constituents of the residue itself) has little effect upon the precipitation index. Therefore, the precipitation index can be determined on a blended fuel just as well as on the residue itself. On mixing two "incompatible" fuels, the precipitation formed is the least soluble material in the mixture, which will normally come from only one of the fuel oils. The precipitation index of the mixed fuel will therefore be the same as that of the fuel containing the least soluble component. On the other hand, although each stable fuel may contain cutter stock that is adequate for its own least soluble component, a blend of the two cutter stocks would have average solvent powers. In the case of "incompatible" fuels, these properties are inadequate for the least soluble asphaltenes in the mixture. Consequently, the basis of the present invention comprises the utilization of these physical observations so as to controllably produce precipitation of asphaltogenic materials for the purpose of subsequent combustion and increase in radiation of the flames so produced.

The residual oil forming the asphaltogenic oil component of the subject fuel oils may be straight run or cracked petroleum residues. Typical species of these

materials include thermally treated asphalt base petroleum residues, which are relatively high in paraffinic materials and have a low precipitation index, uncracked naphthenic residues which likewise have low precipitation indices, mildly cracked asphaltic residues having intermediate precipitation indices and severely cracked residues having relatively high precipitation indices. The residual oils forming the heavier component of the subject fuel oils have precipitation indices greater than 25 or 30 and preferably have precipitation indices bearing between about 35 and about 80. Normally, these will be between about 40 and about 75 and ordinarily it is preferred that fuel oils be combined which have residual oils differing approximately at least about 10 units in precipitation index numbers. In a preferred embodiment, a first residual oil containing an uncracked residual oil possessing a precipitation index of about 30-40 is mixed with a second residual fuel oil containing a cracked residual oil possessing a precipitation index of about 45-80. Residual fuel oils forming the heavy component of the fuels normally have the following characteristics:

Penetration—0 to >1000 (the higher values (500-71,000) from distillation and thermal cracking—the lower values (0-500) from vacuum flashing)  
Softening point—140 to <32° F.  
Flash point—150 to 450° F.

## Typical residues

|                                                                                           | Kuwait<br>Short<br>Residue              | Flasher<br>Pitch    |
|-------------------------------------------------------------------------------------------|-----------------------------------------|---------------------|
| 35                                                                                        |                                         |                     |
| Specific gravity—<br>Softening point, °C—<br>Penetration at 77° F—<br>Viscosity, cks. at— | 1.013<br>32<br>514                      | 1.027<br>61.5<br>10 |
| 75° C—<br>100° C—<br>125° C—                                                              | 3,310<br>538<br>176                     | —<br>4.8<br>5.1     |
| 40                                                                                        | Percent asphaltenes—<br>Percent sulfur— | —                   |

The cutter stocks with which these residual fuels are combined are lower boiling distillate materials normally of petroleum origin which serve the dual purpose of reducing the viscosity of the fuel oil and at the same time maintaining a substantially homogeneous composition. Under previously known circumstances it was believed to be desirable to burn substantially homogeneous fuels so as to prevent plugging of outlet nozzles and the like. Moreover, the uncontrolled and unplanned-for precipitation of asphaltogenic materials results in agglomeration as a sludge which is entirely undesirable and would be useless for operation of the present invention. In order to be successful, the precipitated particles must be formed in a highly dispersed form having an average maximum particle diameter of between about 0.5 and about 150 microns each. Particles smaller than or larger than these desired limits caused reduced amounts of radiation of a burning flame to occur.

The cutter stocks, therefore, which may be utilized in the asphaltogenic residual fuels are those which have a higher solvency index than the precipitation index of the residual oil components of the fuel. This is normally essential in order to produce a homogeneous fuel composition. The solvency index of the most preferred cutter stocks is normally between about 35 and 95 as determined by the procedure given hereinbefore. Suitable cutter stocks include petroleum aromatic extracts, such as furfural extract of catalytically cracked gas oil, Edeleanu extracts of various boiling points such as that from 375 to 590 or from 500 to 650° F., aromatic extracts from flashed pitch, light catalytically cracked gas oil, clarified oil, heavy catalytically cracked gas oil and the like.

Following is a table listing the physical properties of typical specific cutter stocks:

|                            | L.A.<br>Basin<br>Cat.<br>Cracked<br>Gas Oil | L.A.<br>Basin<br>Clarified<br>Oil | West<br>Texas<br>Light<br>Cat.<br>Cracked<br>Gas Oil | West<br>Texas<br>Heavy<br>Cat.<br>Cracked<br>Gas Oil |
|----------------------------|---------------------------------------------|-----------------------------------|------------------------------------------------------|------------------------------------------------------|
| API gravity                | 20.8                                        | 11.0                              | 31.2                                                 | 26.6                                                 |
| Percent sulfur             | 1.08                                        | 1.02                              | 0.32                                                 | 0.70                                                 |
| Diesel index               |                                             |                                   | 41.1                                                 | 42.2                                                 |
| ASTM distillation, °F.:    |                                             |                                   |                                                      |                                                      |
| I.B.P.                     | 425                                         | 454                               | 408                                                  | 488                                                  |
| F.B.P.                     | 715                                         | 760+                              | 470                                                  | 568                                                  |
| 10%                        | 487                                         | 526                               | 514                                                  | 624                                                  |
| 50%                        | 526                                         | 642                               | 574                                                  | 680                                                  |
| 90%                        | 619                                         |                                   | 618                                                  | 700+                                                 |
| Percent recovery           | 98                                          | 85                                | 99.0                                                 | 97.0                                                 |
| Pour point, °F.            |                                             | -5                                | 0                                                    | 55                                                   |
| Percent Ramsbottom carbon  |                                             |                                   | 0.08                                                 | 0.24                                                 |
| Solvency index             | 54                                          | 52                                | 50                                                   | 36                                                   |
| Viscosity, SSU, at 100° F. | 37                                          | 71                                |                                                      |                                                      |
| Aniline point, °F.         | 93                                          | 101                               |                                                      |                                                      |

It will be understood that the residual fuel oils may vary widely in their two components and in the combination of the two components, namely, in the residual fuel itself, in the cutter stock itself and in the combinations which may be made of these two components. For example, with a residual oil having a relatively low precipitation index, such as an uncracked highly paraffinic or an uncracked naphthenic type residual oil, it is possible to select a cutter stock from a much wider variety of distillates than is possible with residual fuels having higher precipitation indices. This is possible since most cutter stocks possess solvency indices high enough to maintain homogeneity with almost all relatively low precipitation index residual oils. However, as the precipitation index of a residual oil increases, the possibility of selection of cutter stocks which will maintain homogeneity therewith becomes more and more restricted. The selection of a cutter stock will depend upon not only the precipitation index of the residual oil but also upon the viscosity, pour point and flash point desired in the final residual fuel oil composition.

The proportion of residual oil to cutter stock in the fuel oil composition will vary within relatively wide limits but normally will be between about 25 and 75% cutter stock, the balance of the composition being the residual oil. Another limitation on the percentage of cutter stock will be the minimum concentration of cutter stock necessary to insure that the individual residual fuel oils will be homogeneous until they are purposely mixed for the object of producing a desired type of particle dispersion just prior to burning.

Having selected the individual initially homogeneous residual fuel oils to be combined for the purpose of precipitation of particles it then becomes necessary to determine the proportion of each oil to be used in order to insure precipitation. This can be readily calculated in accordance with the following method:

A state of incipient precipitation exists when the solvency index of a blend of fuel oils just equals the precipitation index of the most insoluble residue in the blend. This may be stated as follows:

$$\frac{(V_{csa})(S_{csa}) + (V_{csb})(S_{csb})}{V_{csa} + V_{csb}} = S_{blend} = P_{I_h}$$

where:

$V_{csa}$ =volume of cutter stock *a* in the blend.

$S_{csa}$ =solvency index of cutter stock *a*.

$P_{I_h}$ =precipitation index of most insoluble residue in the blend.

Then  $1-X$ =volume fraction of cutter stock *b* in the cutter stock portion of the fuel blend. Then the equation can be rewritten as follows:

$$X(S_{csa}) + (1-X)(S_{csb}) = P_{I_h}$$

Solving for X we have:

$$X = \frac{P_{I_h} - S_{csb}}{S_{csa} - S_{csb}}$$

5 In a practical example the volume fraction (X) of one of the cutter stocks in the cutter stock portion of the blend is first calculated. Then from the cutter stock content of the fuel and the volume fraction X, the actual volume percent of this fuel in the blend is calculated.

10 As an example the calculation for blends of fuels A and B in Table I will be made. The percentage of fuel A required to produce precipitation in the blend will be determined.

$$S_{IA} = 36, S_{IB} = 56, P_{I_h} = 45$$

$$X = \frac{45 - 56}{36 - 56} = \frac{-11}{-20} = 0.55$$

=volume fraction of cutter stock A

20 in the cutter stock portion of the blend. Fuel oil A contains 65.6% cutter stock. Then the volume of fuel oil A in the blend will be

$$\frac{0.55}{0.656} = 0.84 \text{ volume of fuel A}$$

25 Similarly for fuel B the volume fraction of cutter stock B in the cutter stock portion of the blend is  $(1-X)$  or 0.45. Since fuel oil B contains 50% cutter stock the volume of fuel oil B in the blend will be

$$\frac{0.45}{0.50} = 0.9 \text{ volume of fuel B}$$

Then the percent of fuel A in the blend is

$$35 \frac{A}{A+B} \times 100 = \frac{0.84}{0.84 + 0.9} = \frac{0.84}{1.74} \times 100 = 48\%$$

When the amount of fuel oil A in the blend is this amount or greater, precipitation will occur.

Having determined the precipitation index of two fuels and the solvency index of the cutter stocks contained therein, it is possible to calculate the combined composition of the two which will give an assurance of precipitation of particles. In each case, as the working examples given hereinafter will show, it is necessary to mix a sufficient amount of one residual fuel oil with a second and different residual fuel oil in such proportions as to obtain a mixture of cutter stocks having a solvency index which is numerically lower than the precipitation index of the residual oil most prone to precipitate, namely, the residual oil having the highest precipitation index. Under these conditions, precipitation will occur and when the mixed fuel is burned will result in increased radiation thereof.

55 In accordance with a preferred version of the present invention, the precipitated particles (including agglomerates of originally discrete particles) are distributed in particle size over a range from about 0.5 micron to about 150 microns, so that as the relatively smaller particles are consumed and disappear from the flame, the relatively larger particles still persist in acting as radiating bodies. In accordance with one phase of the present invention, this range in particle size of the precipitated particles may be effected by a differential time of particle size existence between several portions of the residual

60 fuel being introduced into the furnace. If, for example, the smallest particles are formed by a residence time outside of the furnace and prior to burning of about 5 seconds or less, then it is preferred that an appreciable portion of the fuel oil be subjected to precipitation techniques for a time prior entrance into the furnace of at least about 30 seconds or more, so that the necessary time for particle growth is gained after which both particle-containing residual fuel streams are introduced, either together or separately, into the flame-burning area.

65 Since it is preferred that substantially continuous ele-

vated emissivity throughout the entire area of the flame is obtained, it is preferred that at least about 10% by weight of the precipitated particles having diameters less than about 0.5 microns and at least 10% by weight of the particles have diameters greater than about 10 microns. Thus, there is virtual assurance that the flame will contain at all times an emission-improving portion of radiating particles, even though the flame be of a length from about several inches to as much as 35 feet. Flames from about 15 to 30 feet are commonly employed in such large scale industrial installations as open hearth steel furnaces and the like. The upper limit of particle size is determined as that size particle which will just be consumed in the particular flame whose length, temperature, percent excess air and linear velocity are known. For any given flame and a knowledge of the furnace geometry this maximum particle size can be determined.

The fuel oils to be treated in accordance with the present invention are defined as being asphaltogenic in nature, by which is meant that said fuel oils are normally residual fuels or contain substantial quantities of residual petroleum components, said residual components comprising in part those bodies of reduced solubility characteristics which have molecular weights above about 1,000, usually 1,000-5,000.

A further improvement in the present invention, especially as applied to situations such as exist in open hearth steel making furnaces, comprises maintaining the flame profile substantially constant during the entire steel making process, and varying the radiation of the flame by controlling the proportion of suitable particles in the fuel stream. A still further improvement in this respect comprises maintaining the total fuel input substantially constant throughout the steel making process, thus maintaining the flame profile substantially unaltered during the same period, but varying the radiation characteristics thereof by variation in particle proportion.

The open hearth furnace is a batch furnace. Steel scrap, pig iron, and sometimes a small proportion of ore are charged to the furnace, melted and refined. In the first stage of the melt, the "charging period," the solids are cold and present an irregular surface to the flame and combustion gases. The actual charge to the furnace is normally carried out in a series of steps since the unmelted mass usually is too large for the entire charge to be made at one time. Consequently, substantially half of the charge is inserted in the furnace and partially or fully melted before further portions of the charge are added. Upon commencement of heating at least a portion of the charge melts sufficiently to substantially submerge the remaining solids and the surface of the charge becomes flat. When this stage has been reached, the so-called "melting period" begins. When the ingredients have all reached the melt stage (or substantially so), the "refining period" starts, during which the liquid charge is maintained at a high and substantially constant temperature for the necessary time to complete purification by separation of the slag from the main body of the melted steel.

It is economically desirable to minimize the time consumed during the charging and melting periods in order to maintain a high rate of production of steel from the furnace. During these first two periods (charging and melting) the temperature is being raised continually and, consequently, during this time the maximum degree of radiation from the flame is desirable. The maximum fuel input rate is limited by the melting temperature of the roof of the furnace as well as the optimum flame profile for efficient transfer of heat from the flame to the melting charge. During the charging period high fuel input rates may be employed when both the charge and the furnace refractory roof are relatively cool. However, during the melting period, the fuel input rate is limited by the maximum allowable temperature of the refractory roof which is ordinarily in the order of 2800-3000° F.

Since the temperature of the charge during this period gradually rises from 2400 to 2600° F., there is a very small margin between required and maximum allowable furnace temperatures.

5 While the fuel input rate can be varied, it will be obvious that the flame profile will alter radically with any change made in this input rate. Hence, it is desirable to establish the optimum flame profile for a given rate of fuel input and thereafter maintain the same rate of total fuel consumption. The present process is based upon these considerations and provides the flexibility necessary for successful operation thereof.

Fuels have been modified in the past by the incorporation of solid fuel materials, especially powdered coal. 15 However, the use of powdered coal in fuel oil suspension does not provide the desired increase in radiant heat, since the powdered coal particles are either relatively extremely coarse and consequently do not present the surface area necessary for optimum black body radiation, 20 or (due to burning rates slower than that of oil) must be ground much finer than precipitated oil particles if they are to be completely consumed. Other solid fuel components used as proposed heretofore, have been incorporated in the entire body of the fuel oil and consequently permitted no latitude in the alteration of the 25 radiation of the flame which must necessarily have remained at a constant value for any total rate of fuel input. Moreover, the principal disadvantage which was experienced with these prior art coal and carbon black 30 suspensions comprised the difficulty of maintenance of the suspension, since in the relatively dilute form in which they are normally employed the particles are not self-supporting and tend to settle out. This property may be overcome in part by incorporation of certain suspending 35 agents and surfactants, but this is an uneconomical means of creating and maintaining the suspensions and also entails certain problems such as the creation of undesirable ash. Since the fuel input into a large furnace such as an open hearth furnace is extremely high, the ash 40 problem becomes serious due to deposition thereof on the sides of the furnace and the operating parts thereof.

The improvement caused by this invention is apparently based upon the increased emission of radiant energy at wave lengths at which solid matter absorbs most efficiently, i.e., in the infra-red range.

The mixture of fuel oils is selected so as to produce precipitated particles in an amount between about 1% and about 10% by weight based on the total fuel.

The effect of increasing the emissivity of the combustion fuels is of great economic significance since it has been ascertained that the average time of completing a run in a standard commercial open hearth furnace can be reduced as much as about 10%.

The addition of the first fuel oil to the second residual fuel oil is preferably effected just prior to injection into the furnace and combustion of the fuel composition. The timing will be adjusted to produce the optimum size of particles in accordance with the limitations set forth hereinbefore but normally will be between about 1 second and 24 hours and preferably between about 30 seconds and one-half hour. The production of particles in a residual fuel, according to the present process, results in substantially spherical particles which, upon aging in the fuel oil composition, tend to agglomerate into larger bodies which still maintain their essentially spherical shape. This is sharply differentiated from the chain-like agglomerates which are created upon the aging of carbon black particles suspended in fuel oils.

In order to maintain a substantially constant supply of 70 radiating precipitated bodies throughout the entire length of a fuel flame such as in an open hearth furnace, it is preferred that the particle size distribution be spread between the limits already stated, namely, between about 0.5 micron and about 150 microns. This may be difficult to attain if the first fuel oil is added to the second

fuel oil at only one particular time prior to combustion of the fuel oil composition. Therefore, in accordance with one phase of this invention, it is a preferred process to inject portions of the first fuel oil into second fuel oil being fed to a burner at two or more time units prior to burning so that an elapsed time is permitted for part of the particles to agglomerate or grow and form the relatively coarser varieties which have a more extended life prior to being completely burnt in the flame during combustion. The two or more portions of the combined fuel may be commingled at the burner or may be injected into the combustion area through separate nozzles. An aging opportunity can be created by passing that portion of the fuel oil in which the relatively larger particles are to be formed into a storage tank preferably containing agitation means or through a coil designed to increase the residence time of the fuel oil therein so as to provide the necessary extended particle formation period prior to burning.

By utilization of the present process of precipitating fuel components in the fuel stream of such furnaces, it has been found that great economic advantages can be obtained, for example, in the cycle time for the production of steel. By the precipitation of 1.5-5% insoluble particles into the fuel oil utilized for the heating of an open hearth furnace, for example, during the charging and melting stages but not during the refining stage, a 10% reduction in total cycle time can be achieved. By maintaining the total fuel input constant during the entire period of steel production (or during any other comparable process, such as cement production) the flame profile was substantially unaltered, but the radiation thereof was radically changed by the injection or omission of the precipitated fuel particles. The increased flame luminosity did not appear to affect refractory life in such furnaces since the temperature of the flame was not substantially different from that of the flame without particle formation. The following examples illustrate the process of the present invention.

The present invention enabled the production of flames of higher radiation from basically low cost residual fuel oils. Thus, it is especially distinguished in this respect from prior art high emissivity compositions wherein materials were added for the purpose of increasing emissivity but only by means of increasing the cost of the total fuel compositions as is true even in the case of the addition of lower molecular weight distillate materials, such as kerosene or gaseous precipitants, such as butane. Consequently, the present invention utilizing the physical properties of precipitating tendencies and limited solvation tendencies of the asphaltogenic materials and of the cutter stock, respectively produces the same desirable degree of increased radiation but at no increase in cost of the total fuel oil components since each of the residual fuel oils has the same basic low price and no premium price materials are involved.

#### EXAMPLE I

Table I which follows shows the properties of four residual fuel oils. Each of the fuels is stable by itself and shows no precipitation of the particles. This is in accordance with the relative precipitation index and the solvency index of the cutter stock in each fuel. It will be noted that the solvency index of the cutter stock in

each case is higher than the precipitation index of the fuel. However, a blend of equal quantities of fuels A and B results in precipitation but combinations of fuels A and C are compatible and show no precipitation of particles in any proportions. A blend of equal quantities of fuels A and D results in a desirable precipitate being formed.

It is possible to predict incompatibility and therefore precipitation of radiation emitting particles of fuel oil blends in advance from the precipitation index values of the residues, the solvency index values of the cutter stocks and the quantity of the cutter stock in each fuel.

Table II which follows shows the results of calculating the solvency index values of blends of equal volumes of various of these four fuels and states the stability or instability of the blend on the basis of data. For example, a 50-50 blend of fuels A and B results in a precipitate being formed. Because the solvency index of the cutter stock in this blend is 39, which is less than the precipitation index of 45 for the least soluble residue in the blend, it is also possible to calculate the minimum amount of fuel A required to cause precipitation of fuel B and this is also shown in Table II to be at least 48% by volume of fuel A blend.

Fuels A and C are stable in all proportions because the lowest solvency index of the pair is higher than the highest precipitation index of the residues in the pair. The same is true of blends of fuels B and C. Blends of fuels A and D result in a precipitate being formed when the blend contains at least 22.5% by volume of fuel A. Fuel oil D may be caused to precipitate by blending with 44% or more of fuels B or C.

The quantity of precipitate formed is roughly proportional to the asphaltene content of the residual fuel and to the difference between the precipitation index of the least soluble residue and the solvency index of the final fuel oil blend. When portions of the blended fuels A and B and of the blended fuels A and D are burned, the resulting flames exhibit substantially increased emissivity due to the formation of the precipitate as compared with the burning of the individual fuels.

Table I

| Type of Residual Fuel Oil...           | A<br>Un-cracked<br>Highly<br>Paraffinic | B<br>Very<br>Mildly<br>Cracked | C<br>Un-cracked<br>Naphthenic<br>Type | D<br>Severely<br>Cracked |
|----------------------------------------|-----------------------------------------|--------------------------------|---------------------------------------|--------------------------|
| API gravity.....                       | 23.4                                    | 16.5                           | 17.6                                  | 6.3                      |
| Penskey-Martens flash, ° F.....        | 260                                     | 190                            | 202                                   | 196                      |
| Viscosity, SSU, at 122° F.....         | 142                                     | 204                            | 197                                   | 199                      |
| Pour point, ° F.....                   | 25                                      | -10                            | -15                                   | -15                      |
| B. S. and W., percent.....             | 0.2                                     | 0.2                            | 0.1                                   | 0.3                      |
| Conradson carbon, percent.....         | 3.3                                     | 9.0                            | 6.9                                   | 15.6                     |
| Ash, percent.....                      | 0.03                                    | 0.03                           | 0.05                                  | 0.08                     |
| Isopentane insoluble, percent.....     | 1.6                                     | 9.9                            | 7.0                                   | 17.4                     |
| Stability to Navy heater test.....     | ( <sup>1</sup> )                        | ( <sup>1</sup> )               | ( <sup>1</sup> )                      | ( <sup>1</sup> )         |
| Precipitation index.....               | 35                                      | 45                             | 33                                    | 77                       |
| Solvency index of cutter<br>stock..... | 36                                      | 56                             | 56                                    | 90                       |
| Percent cutter stock.....              | 65.6                                    | 50.0                           | 50.1                                  | 60                       |

<sup>1</sup> Stable.

Table II

#### STABILITY OF FUEL OIL BLENDS CALCULATED FROM PROPERTIES OF THE FUELS

| Fuel Oil Combinations.....                            | A and B             | A and C                           | A and D                           | B and C                           | B and D                         | C and D                         |
|-------------------------------------------------------|---------------------|-----------------------------------|-----------------------------------|-----------------------------------|---------------------------------|---------------------------------|
| Solvency index of 50-50 blend.....                    | 39.....             | 39.....                           | 62.....                           | 56.....                           | 75.....                         | 75.....                         |
| Precipitation index of least soluble<br>residue.....  | 45.....             | 35.....                           | 77.....                           | 45.....                           | 77.....                         | 77.....                         |
| Stability of 50-50 blend.....                         | Unstable.....       | Stable.....                       | Stable.....                       | Stable.....                       | Unstable.....                   | Unstable.....                   |
| Minimum concentration to insure<br>precipitation..... | At least 48% A..... | Stable in all<br>proportions..... | Unstable<br>At least 22.5% A..... | Stable in all<br>proportions..... | Unstable<br>At least 44% B..... | Unstable<br>At least 44% C..... |

I claim as my invention:

1. A method of improving the radiation emission of asphaltogenic residual fuel oils during combustion thereof which comprises mixing two residual fuel oils, each fuel oil comprising a residual oil and a distillate cutter stock having a solvency index of 35-95, at least one of the residual oils having a precipitation index greater than the solvency index of the combined cutter stocks, said fuel oils being mixed in proportions between about 1:4 to about 4:1 on a volume basis, said proportions being sufficient to precipitate between about 1% and about 10% by weight of the total fuel components as high molecular weight asphaltogenic particles having maximum diameters between about 0.5 micron and about 150 microns, said mixing being effected from about 1 second to 24 hours prior to burning.

2. A method of improving the radiation emission of asphaltogenic residual fuel oils during combustion thereof which comprises mixing a first residual fuel oil having a precipitation index greater than about 25 with a second residual fuel oil, the fuel oils each comprising a residual oil and a cutter stock having a solvency index of 35-95, the combined distillate cutter stocks present in the mixed oils having a solvency index numerically less than the precipitation index of any residual oil component present therein, said fuel oils being mixed in proportions between about 1:4 to about 4:1 on a volume basis, said proportions being sufficient to precipitate between about 1% and about 10% by weight of the total fuel components as high molecular weight asphaltogenic particles having maximum diameters between about 0.5 micron and about 150 microns, said mixing being effected from about 1 second to 24 hours prior to burning.

3. A method of improving the radiation emission of asphaltogenic residual fuel oils during combustion thereof which comprises mixing 25-75% by volume of a first residual fuel oil having a precipitation index of about 45-75 with 75-25% by volume of a second residual fuel oil, both of said fuel oils comprising 50-75% by weight of distillate cutter stock having a solvency index of 35-95, the solvency index of the combined cutter stocks being numerically less than the precipitation index of said first residual fuel oil, whereby between about 1% and about 10% by weight of the total fuel components precipitate as high molecular weight asphaltogenic particles having maximum diameters between about 0.5 micron and about 150 microns, said mixing being effected from about 1 second to 24 hours prior to burning.

4. A method of improving the radiation emission of

5

10

20

25

30

35

40

45

asphaltogenic residual fuels which comprises mixing 25-75 parts by volume of a first residual fuel oil containing an uncracked residual oil possessing a precipitation index of about 30-40, said residual oil being diluted with a distillate cutter stock having a solvency index greater than the precipitation index of the residual oil, with 75-25 parts by volume of a second residual fuel oil containing a cracked residual oil possessing a precipitation index of about 45-80, said residual oil being diluted with a distillate cutter stock having a solvency index numerically greater than the precipitation index of the cracked residual oil, each of the cutter stocks having a solvency index of 35-95, the two fuel oils being mixed in proportions such that the solvency index of the combined cutter stocks is numerically less than the precipitation index of the cracked residual oil, whereby between about 1% and about 10% by weight of the total fuel components precipitate as high molecular weight asphaltogenic particles having maximum diameters between about 0.5 micron and about 150 microns, said mixing being effected from about 1 second to 24 hours prior to burning.

5. A method of improving the radiation emission of asphaltogenic residual fuel oils which comprises mixing at least two residual fuel oils, each comprising a residual oil and a distillate cutter stock, the precipitation index of at least one of the residual oils being 35-80 and the solvency index of each cutter stock being 35-95, each fuel oil being substantially free of precipitated asphaltogenic particles prior to mixing, the two fuel oils being mixed in volume proportions between about 1:4 to about 4:1, said proportions being at least sufficient to produce a mixture of cutter stocks having a solvency index at least about one unit less than the precipitation index of any of the residual oil components present, whereby between about 1% and about 10% by weight of the total fuel components precipitate as high molecular asphaltogenic particles, said mixing being effected from 5 seconds to 24 hours prior to burning, whereby particles having maximum diameters between about 0.5 micron and about 150 microns are formed.

#### References Cited in the file of this patent

#### UNITED STATES PATENTS

|           |                      |               |
|-----------|----------------------|---------------|
| 2,246,760 | Ryan et al. -----    | June 24, 1941 |
| 2,663,675 | Ewell -----          | Dec. 22, 1953 |
| 2,687,991 | Miller -----         | Aug. 31, 1954 |
| 2,755,229 | Beuther et al. ----- | July 17, 1956 |